

## UNITED STATES PATENT OFFICE

2,650,162

## WELD ROD

Arthur T. Cape, Los Angeles, Calif., assignor to  
 Coast Metals, Inc., Little Ferry, N. J., a corpora-  
 ration of Delaware

No Drawing. Application July 31, 1951,  
 Serial No. 239,630

3 Claims. (Cl. 75—125)

**1** This invention relates, as indicated, to weld rods, but has reference more particularly to a weld rod which is especially useful for hard facing parts of equipment used in copper metallurgy, which parts are susceptible to or subjected to the combined effects of corrosion and erosion from molten copper, copper oxide and copper matte.

Among such parts are copper converter lips, ladles, ladle lips, slag pots, and other parts onto which molten copper, copper oxide, or copper mattes may drip and cause wear.

Various alloys have been tried for facing such parts in an effort to combat such corrosive and erosive effects, but none has proven satisfactory, from the standpoint of total life and general utility.

As the result of considerable work which I have done towards meeting this problem, I have developed an alloy which satisfactorily withstands, for long periods, the corrosive and erosive effects of molten copper, copper oxide, and copper matte.

The weld rod of the invention contains from about 24% to about 40% of chromium, from about .5% to about 3% copper, and from .5% to 1.75% carbon, with the balance substantially all iron.

The alloy, in the form of a weld rod, is used for applying a coating or facing thereof to the portion of the equipment or apparatus which is subject to the aforesaid effects, such for example, as the lip of the converter. It will be understood, however, that the alloy may be used for coating or facing portions of other apparatus used in the handling of molten copper, such as the lips of copper holding ladles, the bottoms of ladles upon which the stream of molten copper impinges, etc.

The facing or coating deposited by the rod 40 remains virtually unattacked under the conditions under which it is used, and has an extremely long life. The metal welds without porosity or cracking, a factor which is of extreme importance, because molten copper will seep 45

through cracks or pores and attack the iron base.

The alloy, as thus described, may also be used in the form of castings, in cases where the castings are used outside of the copper converter and are not in contact with white metal, which is Cu<sub>2</sub>S.

It will be understood that slight changes may be made in the analysis without departing from the spirit of the invention, or the scope of the appended claims.

Having thus described my invention, I claim:

1. An alloy which is particularly resistant to the corrosive and erosive effects of molten copper, copper oxide, and copper matte, said alloy 15 containing chromium in amounts of from about 24% to about 40%, copper in amounts of from about .5% to about 3%, and carbon from .5% to 1.75%, the balance consisting essentially of iron.

2. A weld rod which is especially adapted for hard facing parts of apparatus used in copper metallurgy and subjected to the corrosive and erosive effects of molten copper, copper oxide and copper matte, said rod containing chromium in amounts of from about 24% to about 40%, copper in amounts of from about .5% to 3%, and carbon from .5% to 1.75%, the balance consisting essentially of iron.

3. As a facing for apparatus parts subjected 30 to the corrosive and erosive effects of molten copper, copper oxide and copper matte, an alloy containing chromium in amounts of from about 24% to about 40%, copper in amounts of from about .5% to 3%, and carbon from .5% to 1.75%, the balance of the alloy consisting essentially of iron.

ARTHUR T. CAPE.

## References Cited in the file of this patent

Stainless Steels, 2nd edition, page 647. Edited by Thum. Published in 1935 by the American Society for Metals, Cleveland, Ohio.

The Coal Age, vol. 38, No. 10, Oct. 1933, page 341. Published by the McGraw-Hill Publishing Company, New York.